# EUROPEAN PATENT APPLICATION

(11) **EP 4 627 957 A1**
(43) Date of publication of application: **08.10.2025**
(21) Application number: 24168408.3
(22) Date of filing: 04.04.2024
(51) Int. Cl.: A41D 13/015, A41D 13/05, A41D 31/24, A41D 31/28

(54) **GARMENT ARTICLE FOR PERSONAL IMPACT PROTECTION**

(71) Applicant: Freudenberg Performance Materials B.V., 6827 AV Arnhem (NL)
(72) Inventor: CHURKO MONTERO, Sergio, 6827 AV Arnhem (NL); CORTINA CRUZ, Jordi, 6827 AV Arnhem (NL); MADELIN, Axelle, 6827 AV Arnhem (NL); ZIEM, Sarah, 6827 AV Arnhem (NL); ZANETTI, Cristiano, 6827 AV Arnhem (NL); DE JONGE, Hans, 6827 AV Arnhem (NL)
(74) Representative: CPW GmbH

(57) **Abstract**

The application pertains to a garment article for personal impact protection. The garment article comprises at least one shock-absorbing material and at least one flexible two-dimensional material. The garment article is characterized in that the shock-absorbing material is a three-dimensional mat of thermoplastic fibers which fibers are randomly oriented the flexible two-dimensional material covers at least a part of the shock-absorbing material, that the shock-absorbing material is connected to the garment article.

## Description

The invention pertains to a garment article for personal impact protection. Personal protection is one of the main purposes of any kind of garment. The most intuitive function of garment is actually protection of a person's intimacy and protection against cold. However, also protection against mechanical impacts of any kind has always played a role for different kinds of garment. The most remarkable pieces of garment in this sense may be helmets worn by e.g. construction workers or cyclists which are to protect the head and especially the brain against impacts in case of an accident. Also in many kinds of sports helmets and other impact protection garments are present, especially in sports known for intense body contact such as different kinds of football like American, Australian or Canadian football, boxing or wrestling or sports involving rackets, or sports using hard balls or pucks such as cricket, field hockey or ice hockey.

Modern impact protection is frequently based on foam pads which are typically covered with fabric in order to both enclose the foam pads in the garment article and to cover the uncomfortable hand and unattractive look foam pads typically have. Polyurethane (PU) foam is frequently used to manufacture said foam pads as it is readily available, cheap and can be shaped in many different forms. However, foam pads in general and PU foam pads in particular have two major disadvantages. First, foam pads can get soaked by liquids in case of exposure to e.g. rain or sweat, with sweat being of special importance for sports clothing. However, due to their porous structure, foams tend to dry very slowly giving microbes the chance to spread in the foam pad resulting in both hygienic problems and bad odour of the garment.

Third, foam pads provide strong thermal insulation which may become very uncomfortable for the wearer especially in hot environments and/or when carrying out exhausting activities.

Finally, foams and especially PU foams are a big obstacle to recycling which also in the field of garments has become more and more important during recent years. It is thus the object of the present invention to provide a garment article suitable for personal impact protection which is better recyclable and more hygienic compared to the prior art.

The object is achieved by a garment article comprising at least one shock-absorbing material, at least one flexible two-dimensional material characterized in that the shock-absorbing material is a three-dimensional mat of thermoplastic fibers which fibers are randomly oriented, the flexible two-dimensional material covers at least a part of the shock-absorbing material, and the shock-absorbing material is connected to the garment article.

Throughout the present application, the expressions "garment" and "garment article" will be used synonymously. According to the present application, the expression "garment" should be interpreted in the broadest way as possible and include everything which has the main purpose of covering at least a part of the body. Due to this definition, the expression "garment" includes, but is not limited to, articles which are as different as shirts, blouses, overalls, sweaters, jackets, vests, trousers, shorts, boxers, briefs, pants, socks, shoes, hats, caps or helmets but also scarfs or hoods. For the definition as a garment, it is not relevant whether the article is worn directly on the skin as e.g. underwear, over underwear or even in layers further removed from the body, like a jacket which may be worn over a sweater being worn over a shirt. The garment may be used for all different kinds of applications and occasions. The garment may be a piece of business or leisure clothing, a piece of a uniform, a piece of functional clothing used for any kind of sports or a piece of protectional clothing used in any kind of hazardous situation or place. Sports according to the present application is not particularly limited but includes kinds of sports such as games carried out with balls or similar items, like different kinds of football including soccer, handball, basketball, volleyball, rugby, cricket, field hockey, ice hockey, tennis, badminton or table tennis, as well as fighting sports such as boxing, wrestling, karate or judo or other martial arts, but also sports like skiing, different kinds of skating, like roller skating, ice skating, inline skating or skateboarding, snowboarding, cycling, athletics involving running, jumping and/or throwing, swimming, diving, or different kinds of surfing.

The garment according to the present application is explicitly not limited to garment which already by its name is considered a personal protection as its name comprises expression such as "guard" or "protection" as it is e.g. the case for chest guards or the like.

Garment for hazardous situations or places may provide protection against extreme temperatures like against cold, for e.g. expeditions in mountainous areas or polar regions, or against extreme heat, e.g. for work on different kinds of furnaces like in metal, glass or cement industries.

An impact according to the present application means a sudden influence of blunt force to the human body like a shock or a slap caused by violence of a person, a collision with an object or a fall. What is explicitly not covered by the present invention is protection against non-blunt impacts on the human body by e.g. sharp items such as blades or by extremely small and fast items such as bullets or arrows.

The garment according to the present application comprises at least one flexible two-dimensional material. The flexible two-dimensional material may comprise one or several layers of woven or knitted fabric, nonwoven fabric, leather, artificial leather, grid or foil, which layers may be connected to each other by any connection technique known to the person skilled in the art such as sewing, gluing or needling.

In an embodiment, the garment may comprise several layers of flexible two-dimensional material which layers may be different in composition, structure, thickness and/or color. In case a garment article comprises several layers either within one two-dimensional material or several layers of the same or different two-dimensional materials, a layer which faces towards the body of the wearer is called "inner lining" while a layer which is visible on the side of the garment article opposite to the body of the wearer is called the upper material. The optical impression of the garment article is typically dominated by the upper material while the inner lining may play an important role for the way the garment article feels on the body.

"Two-dimensional" according to the present application means that the material has a thickness that is less than three millimeters measured according to EN ISO 9863-1. It is important to notice that the thickness of the flexible two-dimensional material is not necessarily the same as the thickness of the whole garment article which may comprise more than one layer of flexible two-dimensional material and which may furthermore comprise stuffings or fillings in between layers of flexible two-dimensional material like e.g. in a down- or fiber-stuffed jacket.

The term "flexible" should be interpreted as broad as possible in the present application and includes but is not limited to foldability, bendability, stretchability, drapability and any combination of these properties. It is understood that according to the present application, not all these properties must be present for a material to be called flexible. A material can e.g. be flexible when it is essentially not stretchable but shows drapability and foldability like many woven fabrics do.

One function of the flexible two-dimensional material is to cover the three-dimensional mat of thermoplastic fibers, e.g. in order to shield an unattractive look and/or an uncomfortable hand from the wearer of the garment or from the public the garment article is exposed to. In order to serve this purpose, the flexible two-dimensional material may have a certain color, pattern or structure which may provide it with a desired look and/or hand.

When foam pads are used, the problem of uncomfortable hand can be solved by coverage with a thin layer of e.g. fabric which compensates for the roughness and hard grip of the foam. This may not be possible for certain embodiments of the three-dimensional mat according to the present application as the surface of the three-dimensional mat may be less homogeneous and more rough, harder, sharper or more uneven than the surface of a typical foam pad. Thus, the two-dimensional flexible material may not just have to cover a surface but may also distribute forces exerted to the three-dimensional mat or by the three-dimensional mat in such a manner that single fibers of the three-dimensional mat cannot be felt by the wearer of the garment article under the forces that are exerted to the three-dimensional mat during wearing of the garment. In order to serve this purpose, the flexible two-dimensional material has a thickness of at most 3 millimeters and may be a felt, a carded, spunbonded, airlaid or hydroentangled nonwoven of either staple fibers or filaments, a leather, an artificial leather, a woven fabric or a voluminous knitted fabric, such as a knitted fabric produced in the so-called fisherman's rib technique. In an embodiment, the woven or knitted fabric or the nonwoven fabric has a thickness of at least 2 millimeters.

Different layers of flexible two-dimensional material may be of different character. Thus, one layer of flexible two-dimensional material may be thinner than another layer or different layers of flexible two-dimensional material may be composed of different materials.

A three-dimensional mat according to the present application is a piece of randomly oriented and intermingled fibers which has, in contrast to the flexible two-dimensional material, a thickness of 3 millimeters or higher.

Throughout the present application, it is understood that the terms "three-dimensional mat", "mat" and "three-dimensional mat of thermoplastic fibers" are used synonymously unless it is either mentioned otherwise or unambiguously clear from the context.

In contrast to the flexible two-dimensional material, the three-dimensional mat has the form of a geometric body such as a cuboid, a cylinder, a pyramid, a tetraeder or a cone, or a part or fragment of said geometric bodies such as a truncated cone or a truncated pyramid. In an embodiment, the mat may have a geometric form that that is adapted to the contours of the garment article or the contours of a part of the garment article.

In contrast to the flexible two-dimensional material, the three-dimensional mat of thermoplastic fibers has a remarkable resiliency which enables to use the mat as a shock-absorbing material. Resiliency means that the material upon influence of a pressure, reduces its thickness and restores, at least partly, its thickness after the pressure is released. By compressing, mechanical energy is absorbed in a reduction of thickness and stored in the three-dimensional mat as tension. After release of the pressure, energy is released again by restoring, at least partly the shape and/or the thickness of the three-dimensional mat.

The compression stress of the three-dimensional mat, i.e. the force the mat exerts upon compression, is a measure for the shock absorption property of the three-dimensional mat. Typically, the compression stress is measured at a compression to 70% of the thickness according to DIN EN ISO 3386-1. This norm is typically intended for the examination of foam-like materials but is also used for the examination of three-dimensional fibrous mats.

In an embodiment, the compression stress of the three-dimensional is at most 30 kPa, at most 25 kPa, at most 20 kPa; at most 15 kPa, at most 10 kPa or at most 5 kPa.

In an embodiment, the compression stress of the three-dimensional mat at 70% compression is at least 20 kPa, at least 15 kPa, at least 10 kPa, at least 5 kPa or at least 2 kPa.

As the three-dimensional mat may look unattractive and can have an uncomfortable hand, it is at least in part covered by the two-dimensional flexible material. In an embodiment, the three-dimensional mat is entirely covered by the two-dimensional material and thus has the shape of a pad or a pillow. In such case, the thermoplastic fibers of the three-dimensional mat are entirely concealed from exposure to a user which means that a person does not see the thermoplastic fibers of the three-dimensional mat and may, during normal wearing of the garment article, also do not feel the thermoplastic fibers. Concealing the three-dimensional mat from the user may be realized in several manners.

In an embodiment, the three-dimensional mat may in part be covered by the flexible two-dimensional material.

In an embodiment, a part of the three-dimensional mat is neither covered by the flexible three-dimensional material nor by any material else and is visible on the outside of the garment as a matter of design.

In an embodiment, the three-dimensional mat is covered by a rigid material at the outside of the garment article. Said rigid material may be a plate or a shield. A rigid material according to the present application is material which cannot be folded or stretched without being destroyed and is of a limited bendability. Typical rigid material are shells, plates or grids of resin or metal where the term "resin" includes all kinds of resin known to the person skilled in the art such as thermoplastic resins such as polyamides or acrylo-styrene-butadiene copolymer but also thermosetting resins such as expoxide resins. Fiber-reinforced resins are explicitly included, especially glass- or carbon fiber reinforced resins.

In an embodiment, the rigid material is coated with a lacquer or varnish for corrosion protection and/or decoration.

In an embodiment, the three-dimensional mat may be located in between two layers of the material of the garment article, which layers may be the upper material and the inner lining, may be flexible or rigid and may be fixedly or removably connected thereto. It is understood that these embodiments may be combined with each other in such a way that the three-dimensional mat is fully covered by the two-dimensional material or by the two-dimensional material and the rigid material. The three-dimensional mat may be connected to the material of the garment article or may be located in between two layers of the material of the garment article and may be fixedly or removably connected thereto.

According to the present application the term "connected" means that two items may be either fixedly or removably connected to each other. "Fixedly connected" according to the present application means that two items are connected to each other in such a way that they cannot arbitrarily be fixed to and removed from each other, but that removal means that a connection is irreversibly destroyed. Typical examples for fixed connections according to the present application are connections by sewing or by gluing. It is understood that a connection by sewing does not only include the case where there is a stitching directly connecting the two items such as the mat and the two-dimensional material but also cases where an item is enclosed between two layers which layers are sewn together in such a manner that they form a completely closed pocket wherein an item such as the three-dimensional mat, is enclosed without the item itself being sewed or glued to the upper material and/or the inner lining of the garment article.

In an embodiment, the mat may be enclosed between two layers of two-dimensional material but is, at the same time, fixedly or removably connected to one of the layers or to both layers of two-dimensional material by e.g. stitching, sewing, gluing or using Velcro connectors.

"Removably connected" according to the present application means that two items are connected to each other in such a manner that they can be fixed to each other and disconnected from each other essentially without any damage apart from wear. Removable connections are e.g. connections by Velcro connectors, zippers or with the item being put into a pocket which is formed by two layers of material belonging to the garment article which pockets can be closed and opened e.g. by a lug of material, Velcro connectors, buttons, hooks and loops, or a zipper or any combination thereof.

The garment article according to the application is not particularly limited, however, in an embodiment it can be a garment article such as a cap, a hat or a helmet used in dangerous work environments such as construction zones, factories or harbour areas, but also in sports such as cycling, skiing, horseriding, snowboarding or skating. Also helmets used in motorcycling are covered by the present application. Especially if the garment is a helmet, it typically comprises a shell of rigid material on the outside.

In an embodiment, the garment article is a headgear as it is used in boxing to protect the head and the brain from impact.

In an embodiment, the garment is a type of protection wear worn for certain kinds of dangerous sports such as MX cycling, cricket or different kinds of hockey. The garment may then be a chest guard, neck guards, shin guards, elbow pads or shoulder pads.

In an embodiment, the garment article is a jacket especially suited for shock protection such as a jacket worn in cycling or motorcycling, or by military, police or security personnel.

In an embodiment, the garment article is a glove to protect either the wearer or any other person from shocks or impacts such as a boxing glove, a glove worn in certain kinds of sports such as by football players, especially goalkeepers, baseball or field hockey or ice hockey players. It is understood that the term "glove" according to the present application includes the term "mitt".

In an embodiment, the garment article is a jock cup worn for protection of genitals. Typically, a jock cup is a hard-shell or cushioned inlay worn in a pouch integrated into the underwear, typically in a so-called jockstrap but also in briefs, boxers or hipsters.

In an embodiment, the garment article can be a chest protector. Chest protectors are typically worn to protect the chest area. In an embodiment, the chest protector may be a bra. In an embodiment, the bra may comprise shock-absorbing bra-cups.

In an embodiment, the garment article is a belt as e.g. worn in motorcycling as shock protection for the kidneys.

In an embodiment, the garment article is an overall which may be an overall worn on the upper body, on the lower body or a one-piece overall covering the whole body. According to the present invention, the lower body is the part of the body which is below the waist while the upper body is the part of the body which is over the waist. Garment articles which cover the whole lower body may also reach over the waist, however, they do not cover the whole upper body. The same holds true for garment articles which cover the upper body and which may reach underneath the waist, however, they do not cover the whole lower body. Overalls like this may be used as shock protection e.g. in water sports such as canyoning or different kinds of surfing.

The garment article may be trousers. Unless otherwise stated, the expression "trousers" according to the present application comprises all kinds of clothing worn from the hips downwards such as regular trousers, boxers, shorts or pants independent of whether they are worn directly on the skin or as upperwear. In trousers, the three-dimensional mat may be comprised in any part of the trouser such as in the rump, in the legs or in the knees.

In an embodiment, the garment article may be a shoe. In a shoe, the three-dimensional mat may be comprised in any part of the shoe depending on the kind of impact the shoe should protect against. Thus, the three-dimensional mat may be part of the sole, e.g. in a running shoe, of the toe section or of the upper material.

In an embodiment, the flexible two-dimensional material may be a nonwoven fabric such as a felt, a carded, spunbonded, airlaid or hydroentangled nonwoven of either staple fibers or filaments, a leather, an artificial leather, a woven fabric or a voluminous knitted fabric.

In an embodiment, the two-dimensional material is a part of the inner lining and/or of the upper material of the garment article. In an embodiment, the flexible two-dimensional material is a part of the garment article that is not visible to the user as it may completely be covered by the inner lining, the upper material or by any combination thereof.

As the mat is a three-dimensional body, it has three different dimensions. Typically, the smallest of these three is called "thickness". The plane spanned by the two largest dimensions is called "surface area" throughout this application. The three-dimensional mat of thermoplastic fibers may be a construction that is essentially open. "Essentially open" according to the present application means that the mat is of a character, that the fibers comprised in the mat form a framework which surrounds a space which is essentially empty or filled by a gas such as air, respectively, in such a manner that the volume of the mat exceeds the volume of the fibers comprised therein by a multiple. In an embodiment, the mat comprises at least 50 Vol.-%, at least 80 Vol.-%, at least 90 Vol.-% or at least 95 Vol.-% of gas or open space, respectively. The amount of empty space is determined by the relation between the density of the mat and the density of the material of the fibers. In both cases, the density is the ratio between the weight and the volume.

In an embodiment, the amount of empty space comprised in the mat is so large that it is possible to see through the mat with a human eye although it may have a thickness of several centimeters.

The amount of empty space in a unit volume of the mat is larger than the same volume of a foam. This reduces the amount of liquid, the mat can absorb compared to a foam. This is not only an advantage over foam-like materials but also over three-dimensional knitted materials which also have a lower amount of empty space per unit volume compared to three-dimensional mats. In comparison to foams and knitted materials a three-dimensional mat according to the present application thus provides the best ventilation effect.

The larger the amount of open space in the mat is, the better is the mat's ability to dry after exposure to liquids such as rain or sweat which enables improvement of the hygienic properties of the garment article.

Another unexpected effect of the larger empty space of the garment article according to the present application is an improved ventilation. Through the large amount of empty space, air may circulate and thus not only provide better drying and thus a hygienic benefit but also transport heat which may accumulate under the garment article so that wearing the garment article becomes more comfortable for the wearer.

In an embodiment, the empty space of the garment according to the present application may be used for active ventilation by air or gasses which may flow through the garment with the air or the gasses being either heated to warm up the wearer in a cold environment or to cool the wearer down in a warm environment or while carrying out exhausting work or sports.

In an embodiment, the empty space may comprise plastic tubes through which water or another liquid is flowing for either warming up or cooling down the wearer. In an embodiment, the mat has an areal weight of at least 200 and at most 1500 g/m². In an embodiment, the areal weight of the mat is at least 400, at most 600 g/m², at most 800 g/m², at most 1000 g/m² or at most 1200 g/m².

In an embodiment, the mat has a residual thickness of at least 70%, at least 80% or at least 90% of the original thickness after 1000, 5000, 10000, 50000 or 80000 compression cycles and a residual compression hardness at compression of 25% of at least 70%, 80% or 90% of the original compression hardness at 25% compression after 1000, 5000, 10000, 50000 or 80000 compression cycles according to DIN EN ISO 2439, method A.

In an embodiment, the compression hardness of the mat is the same over the whole surface area of the mat. In an embodiment, the compression hardness of the mat varies over the surface area of the mat.

In an embodiment, the mat has an air permeability perpendicular to its thickness of at least 10 l/(m²·s), at least 100 l/(m²·s), at least 500 l/(m²·s) or at least 1000 l/(m²·s) at 200 Pa and a pressure gradient of 0.5 measured according to EN ISO 9237.

In an embodiment, the mat has an air permeability parallel to its thickness of at least 10 l/(m²·s), at least 100 l/(m²·s), at least 500 l/(m²·s) or at least 1000 l/(m²·s) at 200 Pa and a pressure gradient of 0.5 measured according to EN ISO 9237.. The air permeability is a property of the mat which makes an important contribution to the ability of the garment article to dry after it has been exposed to liquids such as rain or sweat and which allows for the improvement of the hygienic properties of the garment article.

The three-dimensional mat of thermoplastic fibers may be provided by any suitable process. Preferably, the three-dimensional mat of thermoplastic fibers is provided by extruding polymeric filaments and collecting the extruded filaments into a three-dimensional structure by allowing the filaments to bend, to entangle and to come into contact with each other, preferably in a still molten state or at least in a state where they are still sticky. In an embodiment, the thermoplastic fibers forming the mat may be welded where they cross. In an embodiment, bending and entangling of the extruded filaments are initiated by collecting the filaments onto a profiled surface, which defines the structure of the three-dimensional structured mat of extruded entangled filaments.

In an embodiment, the surface on which the filaments are collected is profiled such that the three-dimensional structured mat of filaments is shaped into a three-dimensional form which comprises structures such as hills and valleys, hemispheres, positive and/or negative cuspates, cups and/or waffles, pyramids, U-grooves, V-grooves, cones and/or cylinders capped with a hemisphere.

In an embodiment, the mentioned shapes are arranged in rows or columns in the three-dimensional mat. V-grooves and U-grooves may extend over a whole row or column such that a row or column may be interpreted as a wave crest and the trench separating two rows from each other may be interpreted as a wave trough. In an embodiment, the surface on which the polymer is extruded, is a profiled rotating drum. In an embodiment, the surface on which the polymer is extruded is a profiled conveyor belt.

In an embodiment, the mat is produced by extruding the polymer melt into a water tank wherein it is formed by two vertical conveyor belts.

In an embodiment, the three-dimensional mat may - apart from the three-dimensionally profiled part, comprise a second part which is two-dimensional and which covers one side of the three-dimensionally profiled part. It is important to notice that, although this part is two-dimensional, it is a part of the three-dimensional mat according to the present application and not a part of the two-dimensional material according to the present application.

The thermoplastic fibers comprised in the three-dimensional mat are not particularly limited to any material but may comprise any thermoplastic polymer known to the person skilled in the art such as polyolefins like polyeythylene or polypropylene, polyamides such as polyamide-6, polyamide-6.6, polyamide-4.10 or polyamide-10.10, polyamide-11, polyesters such as polyethylene terephthalate (PET), polytrimethylene terephthalate (PTT), polybutylene terephthalate (PBT), polynaphylene terephthalate (PNT) or any blends thereof or any copolymers comprising monomers of the named polymers. In an embodiment, the mat comprises a thermoplastic elastomeric polymer. Thermoplastic elastomers may e.g. be of the polyester-ester type or of the polyether-ester type. In an embodiment, the thermoplastic elastomer is polyether block amide (PEBA).

The fibers in the mat may be macroscopic fibers. Macroscopic fibers according to the present application are fibers which a have length of at least 1 centimeter and a apparent diameter of at least 0.25 millimeters. Macroscopic fibers may have the appearance of wires.

In an embodiment, the fibers, be it macroscopic fibers or fibers in general, are filaments. Filaments are fibers which have a length which is essentially infinite compared to their apparent diamenter. Filaments may thus have lengths of several meters or even several kilometers.

The fibers may be massive or hollow. Also combinations of hollow and massive fibers in one mat are possible. Such combinations allow for an adjustment of the compression hardness over the surface area of the mat.

The cross section of the fibers, be it macroscopic fibers or fibers in general, may have any geometry known to the person skilled in the art such as round, oval, oblong or triangular.

In an embodiment, fibers forming the mat have an apparent diameter of at least 0.25 millimeters, 0.35 millimeters or 0.45 millimeters. They may have an apparent diameter of at most 0.55 millimeters, 0.65 millimeters, 0.8 millimeters, 1 millimeter or 1.5 millimeters.

The mat has a thickness of at least 3 millimeters. In an embodiment, the mat has a thickness of at least 4 millimeters or at least 8 millimeters. In an embodiment, the mat has a thickness of at most 23 millimeters, 40 millimeters or 50 millimeters. All mentioned thicknesses of the mat are measured according to EN ISO 9863-1. In an embodiment, the thickness of the mat may vary over its surface area.

In an embodiment, the three-dimensional mat and the flexible two-dimensional material are made from polymers of the same polymer family. Throughout the present application, a polymer family is a group of polymers which are formed from chemically similar monomers. Examples for polymer families are polyolefins, polyamides or polyesters.

In an embodiment, the three-dimensional mat and the flexible two-dimensional material are made from the same polymer.

Providing the three-dimensional mat and the flexible two-dimensional material from the same or similar polymers is beneficial for the recyclability of the garment article.

Recyclability is improved in embodiments where the whole garment article - including the flexible two-dimensional material and the three-dimensional mat - is made from polymers from the same polymer family or even from the same polymer.

In the latter case, it would be possible to recycle the whole garment article without having to separate it into parts depending on the polymer and/or polymer families the parts comprise.

The application further pertains to the use of a three-dimensional mat of thermoplastic fibers as impact-absorbing material in a garment article. It is understood that all considerations made earlier both concerning the garment article and the three-dimensional mat also hold for this aspect of the application. In an embodiment, the thickness of the three-dimensional mat may vary over the surface area. This allows for better adjustment of the resiliency of the three-dimensional mat. The thickness variation may be achieved by stacking more than one three-dimensional mat with the three-dimensional mats that have been stacked may have different surface areas.

The thickness variation may also be achieved by removal of parts of the thickness of the three-dimensional mat e.g. by mechanical and/or abrasive techniques such as milling, skiving or cutting or by thermal techniques which means that parts of the three-dimensional mat are heated to a plastic state and then compressed. Furthermore, the variation of thickness may already be implemented to the three-dimensional mat during the manufacturing process.

In an embodiment, the three-dimensional mat may be of variable density which means that the density of the three-dimensional mat varies over its surface area. This density variation may allow for adjusting the resiliency of the three-dimensional mat as mats of different densities may have different resiliencies. A mat which has variable densities may show variable resiliency with, at the same time, constant thickness.

### Example - Measurement of the compression stress of a three-dimensional mat

Compression stress was measured according to DIN EN ISO 3386-1 on six different samples of three-dimensional mats which can be used in garment according to the present application. The compression stress in kPa as a function of the compression to % of the original thickness is shown in Fig. 1 for six different samples which samples are listed in Tab. 1 together with the compression stress at 70% and 40% compression.

The three-dimensional mat samples consisted of one structured part with a three-dimensional texture, called "profile" and one two-dimensional part directly connected to the three-dimensional textured part called "flatmat". It is important to stress that the two-dimensional part is a part of the three-dimensional mat according to the present application and not of the two-dimensional flexible material according to the present application.

| Name | 70% Compression | 40% Compression | Thickness | Weight | Density | Profile Material | Flatmat Material |
|---|---|---|---|---|---|---|---|
| | [N] | [N] | [mm] | [g/m²] | [kg/m³] | | |
| M21 | 21,24 | 4,66 | 18,9 | 600 | 18 | EL 550-08 | EL250 |
| M22_ | 11,3 | 1,7 | 27,3 | 700 | 26 | EL 550-08 | EL 550-08 |
| M24_ | 7,76 | 1,27 | 18,7 | 300 | 27 | EM400 | EM400 |
| M25_ | 5,9 | 1,18 | 18,9 | 700 | 27 | EM400 | EM400 |
| M20_ | 4,74 | 1,41 | 17,1 | 300 | 18 | EL 550-08 | EL250 |
| M23_ | 1,51 | 0,45 | 24,3 | 300 | 12 | EL 550-08 | EL250 |

The materials EL-550-08, EL 250 and EL 400 are thermoplastic elastomers based on copolyester available under the Arnitel^{®} brand by DSM.

The samples M24 and M25 have been measured as two mats comprising a profile and a flatmat stacked over each other.

## Claims

1. Garment article for personal impact protection, the garment article comprising
• at least one shock-absorbing material,
at least one flexible two-dimensional material **characterized in that**
• the shock-absorbing material is a three-dimensional mat of thermoplastic fibers which fibers are randomly oriented
• the flexible two-dimensional material covers at least a part of the shock-absorbing material,
• that the shock-absorbing material is connected to the garment article.

2. The garment article of claim 1 wherein the garment article is a hat, a helmet, a headgear, a jacket, a glove, a jock cup, a chest protector, a belt, an overall, trousers or a shoe.

3. The garment article of claim 1 or 2 wherein the flexible two-dimensional material is a woven fabric, a knitted fabric, a nonwoven, a leather or an artificial leather.

4. The garment article of any one or more of the previous claims wherein the three-dimensional mat comprises an open space of at least 50 Vol.-%, preferably at least 80 Vol.-%, more preferably 90 Vol.-% and even more preferred at least 95 Vol.-%.

5. The garment article of any one or more of the previous claims wherein the thermoplastic fibers comprise a polyolefin such as polyethylene, polypropylene, a polyamide such a polyamide-6, polyamide-6,6, polyamide-11, polyamide-10,10, polyamide-4,10 or a polyester such as polyethylene terephthalate (PET), polytrimethylene terephthalate (PTT), polybutylene terephthalate (PBT), polyethylene naphthalate (PEN) or a thermoplastic elastomer such as polyether block amide (PEBA).

6. The garment article of any one or more of the previous claims wherein the flexible two-dimensional material consists of a polymer of the same polymer family, preferably of the same polymer, as the three-dimensional mat of thermoplastic fibers.

7. The garment article of claim 6, wherein the whole garment article consists of polymers from the same polymer family, preferably consists of the same polymer.

8. The garment article of any one or more of the previous claims wherein the garment also comprises a rigid material.

9. The garment article of any one or more of the previous claims wherein the three-dimensional mat of thermoplastic fibers comprises three-dimensional structures which are arranged in parallel columns and/or rows.

10. The garment article of claim 9 wherein the three-dimensional structures comprise hemispheres, domes, pyramids, truncated pyramids, cones, truncated cones, cylinders, tetraeders, truncated tetraeders or hexagonal prisms.

11. The garment article of any one or more of the previous claims wherein the thermoplastic fibers are welded where they cross.

12. The garment article of any one or more of the previous claims wherein the three-dimensional mat of thermoplastic fibers is of variable thickness.

13. The garment article of any one or more of the previous claims wherein the three-dimensional mat of thermoplastic fibers is of variable density.

14. Use of a three-dimensional mat of thermoplastic fibers as impact-absorbing material in a garment article.
